

# UNITED STATES PATENT OFFICE.

JOSEPH HEAD, OF HORNELLSVILLE, NEW YORK.

## PROCESS OF TANNING HIDES.

SPECIFICATION forming part of Letters Patent No. 257,442, dated May 2, 1882.

Application filed December 6, 1881. (No specimens.)

*To all whom it may concern:*

Be it known that I, JOSEPH HEAD, a citizen of the United States, residing at Hornellsville, in the county of Steuben and State of New York, have invented certain new and useful Improvements in Processes of Tanning Hides, of which the following is a specification.

My invention relates to a process of tanning hides; and it consists in the following steps 10 or separate portions of the entire process, which are carried into effect in the order set forth, and particularly designated in the claim.

The first step consists in soaking the hides, as they are removed from the animal, in a vat 15 of water about eight feet long, four feet wide, and four feet deep, into which has been poured a mixture of one-half pound of saltpeter, one pound of potash, one pound of oil of vitriol, and twenty pounds of rock-salt. This solution 20 preserves the hides from decomposition, prevents the gelatine from dissolving, and assists in the liming process. They remain in soak from one to two hours.

The second step consists in fleshing the hides 25 after they have been soaked.

The third step consists in placing the hides in a vat of water of about the dimensions given above, into which has been poured a mixture of one bushel of quicklime and one and one-half 30 pound of sal-soda. By the use of this mixture the time necessary to lime the hides is shortened to about six hours. This solution rapidly removes the albuminous substances which hold the hair, but preserves the gelatine 35 intact.

After the hides have been taken from the lime above described, they are ready for the fourth step, which consists in soaking them in a vat of water at a temperature of about 110° 40 Fahrenheit. They are allowed to remain in this vat about two hours, though a shorter time will accomplish the purpose as well.

The fifth step consists in removing the hair and lime-shaving the hides.

The sixth step consists in scouring them upon the grain side to remove all foreign substances, and prepares them for the coloring-liquor. It is seen that after the hides have been lime-shaved they are not placed in a bate, as is usually done, but are immediately scoured. This method I have discovered prepares them for the tan better than the process in common use.

The seventh step consists in coloring the hides. To do this they are placed in a coloring-liquor colored by the different substances 55 well known among tanners. The hides remain in this liquor until they have acquired the desired color, which can be ascertained by watching them. They are immediately scoured when taken out, which removes all sediment and unnatural grain, and constitutes the eighth step 60 of the process.

The ninth step consists in applying the tanning solution. To do this the hides are spread out upon a table or floor and the solution well 65 rubbed in with a swab or brush. The hides are next laid away in a pile, which is the tenth step. They remain in the pile from two to fifteen days, according to the character of the leather to be tanned. While in the pile the 70 hides are handled once a day or oftener, more of the solution applied, and the hides returned to the pile. If, however, it is desired to retain the color upon either side of the hide, the tanning solution is applied to the opposite side 75 from that upon which the color is to be retained, the solution is well boarded in upon that side, the hides folded together separately with the side which is to retain the color outward, and replaced in the coloring solution. 80 If it is desired to retain the color upon both sides of the hide, the tanning solution is applied to both sides, is well boarded in, the hides spread out flat, and returned to the coloring-liquor. The hides remain in this liquor 85 from two to fifteen days, according to the character of the leather to be tanned. While undergoing this process the hides are handled once or twice a day, scoured, more of the solution applied, and returned to the liquor. 90

The eleventh step, which consists in sammying the hides, is then carried into effect.

The twelfth step consists in scouring them on both sides, the thirteenth step in setting them out on a table or floor and flattening them with 95 a slicker, and hanging them up to dry. When the hides have become dry they are taken down, placed upon a table or floor, and stuffed, which constitutes the fourteenth step.

The fifteenth step is then carried into effect, 100 and consists in packing the hides down in a pile and covering them up to protect them from currents of air and from the light, which allows the stuffing to penetrate them without injury

to the color. The length of time the hides remain in the pile is optional, though the shortest time necessary to obtain good results is two hours.

5 The sixteenth step consists in dipping the hides singly in a vat of water at a temperature of about 120° Fahrenheit, which completely drives in all the stuffing previously applied. After the hides have been dipped they are immediately struck out and hung up to dry, which is the seventeenth step.

The eighteenth step consists in whitening, trimming, and boarding them after they have dried, and by which they are made ready for 15 the blacking.

The nineteenth step consists in blacking the hides. I do this with a composition of one pound of lamp-black, one and one-half pound of Babbitt's soap, boiled together in three gallons of water. The advantages I gain by this composition are that it softens and improves the texture of the leather, or, in other words, makes it "mellow." I have discovered that Babbitt's soap gives the best results for this 25 purpose.

The twentieth step is then carried into effect, and consists in smutting the hides off and applying oil and gum-tragacanth to them.

The twenty-first step consists in glassing 30 them down and hanging them up to dry.

The twenty-second step completes the process, and consists in gumming them off with clear gum-tragacanth after they have dried.

What I claim is—

35 The process of tanning hides herein described, consisting of the following steps, which succeed each other in the order designated: first, placing the hides in a vat of water into which has been poured a mixture of one-half 40 pound saltpeter, one pound oil of vitriol, one pound potash, and twenty pounds rock-salt; second, fleshing the hides after they have been soaked; third, soaking them in a vat of water

into which has been poured a mixture of one bushel of quicklime and one and one-half 45 pound of sal-soda after they have been fleshed; fourth, soaking the hides in a vat of water at a temperature of about 110° Fahrenheit after they have been limed; fifth, removing the hair and lime-shaving the hides; sixth, scouring 50 the hides immediately after the hair is removed and they have been lime-shaved; seventh, coloring them; eighth, scouring the hides after they have been colored to remove all sediment and unnatural grain; ninth, the application of the tannin; tenth, laying the hides away in a pile after the tannin has been applied; eleventh, sammying them after they have been tanned; twelfth, scouring them on both 55 sides; thirteenth, setting them out with a slicker and hanging them up to dry; fourteenth, stuffing them after they have become dry; fifteenth, packing them in a pile and covering them up after they have been stuffed; sixteenth, dipping them singly in a vat of water at a temperature of about 120° Fahrenheit after they have been taken from the pile; seventeenth, striking them out and drying them after they have been dipped; eighteenth, whitening, trimming, and boarding them after they have dried; 70 nineteenth, blacking them with a composition of one pound of lamp-black, one and one-half pound of Babbitt's soap, boiled in three gallons of water; twentieth, smutting them off and applying gum-tragacanth and oil after 75 they have been blacked; twenty-first, glassing them down and drying them; twenty-second, gumming them off with clear gum-tragacanth after they have dried.

In testimony whereof I affix my signature in 80 presence of two witnesses.

JOSEPH HEAD.

Witnesses:

HORACE BEMIS,  
D. L. BENTON.